

Patented Apr. 14, 1925.

1,533,798

# UNITED STATES PATENT OFFICE.

BENNETT GROTTA, OF TAMAQUA, PENNSYLVANIA, ASSIGNOR TO ATLAS POWDER COMPANY, OF WILMINGTON, DELAWARE, A CORPORATION OF DELAWARE.

## SECONDARY CHARGE FOR COMPOUND DETONATORS.

No Drawing.

Application filed March 1, 1923. Serial No. 622,208.

To all whom it may concern:

Be it known that BENNETT GROTTA, a citizen of the United States, residing at Tamaqua, in the county of Schuylkill and State 5 of Pennsylvania, has invented certain new and useful Improvements in Secondary Charges for Compound Detonators, of which the following is a specification.

My invention relates to improvements in 10 that type of detonator commonly known as a compound detonator and relates particularly to the main or secondary charge.

The history of modern commercial detonators dates back to the discovery that fulminate of mercury could be employed for 15 initiating nitroglycerine explosives. To this day fulminate of mercury has found universal application as a detonator composition. Early in the development of modern explosives it was found that the efficiency of fulminate of mercury could be increased by the admixtures therewith of a certain class of compounds which, in themselves were not suited for initiating 20 purposes and which in some cases were not even explosive when used alone. These materials are rich in oxygen and are usually termed oxygen carriers. Their admixture is usually so controlled as to supply the deficiency of oxygen in the fulminate of mercury molecule, i. e., supply sufficient oxygen 25 to enable all the carbon present to be converted into carbon dioxide and all the hydrogen present to be converted into water 30 when the mixture is detonated. Various compounds have been used for accomplishing this purpose, such as different metal oxides, perchlorates and chlorates, but of these the chlorate of potassium has probably been used more extensively than all 35 others.

It is well recognized that the problems presented in the production of satisfactory detonator charges are quite different from 40 those existing in the field of general explosives and that apparently slight changes in proportions and in the ingredients frequently produce surprising differences in result.

In recent years efforts have been made to 45 perfect what is commonly known as a compound detonator. A part of the fulminate charge is replaced by any one of a large number of nitroaromatic compounds suitable for the purpose. The detonator is so

constructed that the nitroaromatic compound is itself initiated by the detonation of the fulminate charge which is commonly known as a priming charge. More recently 50 priming charges containing heavy metal azides have been proposed.

In the field of commercial detonators it is universally agreed that the properly constructed compound detonator greatly exceeds the ordinary fulminate composition 65 detonator in initiating efficiency. The general application of this type of detonator has been greatly restricted, however, due to greater manufacturing costs as compared with ordinary fulminate composition 70 detonators. Despite the substitution of a less costly material, i. e., a nitroaromatic compound for a part of the fulminate charge, the ultimate cost of detonators thus charged is ordinarily no less and is usually greater 75 than that of ordinary fulminate composition detonators. This is due to the increased number of operations required for the so-called compound detonators and also to the added expense of specially constructed 80 detonator shells which are usually required.

I have found that not only may oxygen carriers be mixed with primary detonating explosives such as fulminate of mercury without impairing the efficiency thereof but a 85 similar admixture may also be made with any of the secondary nitroaromatic charges with equally gratifying results.

I have found that mixtures of tetrani-troaniline or trinitrophenylmethylnitro- 90 amine, commonly known as tetryl and any suitable oxygen carrier have a detonating efficiency equivalent to and in some proportions greater than that of the original nitroaromatic compound. I have also found that 95 such compositions are approximately equivalent to the original nitroaromatic compound in question, with respect to:

(a) Actual strength as measured by any 100 of the well known tests.

(b) Brisance, as measured by the usual tests for determining this property.

(c) Size of priming charge required for initiation.

(d) Velocity of detonation. 105

By suitable oxygen carrier I mean any solid compound rich in loosely combined oxygen and of sufficient stability to yield a composition that may be safely charged in detonators with other explosive ingredients. 110

ents. Examples of suitable oxygen carriers are ammonium perchlorate, potassium perchlorate and potassium chlorate. Ammonium chlorate and ferric oxide are examples of unsuitable oxygen carriers; ammonium chlorate because of its lack of stability, and ferric oxide because its oxygen content is too firmly fixed to enter into the explosive reaction.

10 Thus my invention constitutes a distinct advancement in the art of initiating explosives by rendering feasible the production of compound detonators with their well known advantage over ordinary detonators.

15 The following examples illustrate the application of my invention:

1. A main charge consisting of 0.5 gram of a mixture of equal parts of tetryl and ammonium perchlorate is charged and pressed into an ordinary detonator shell. This secondary charge is then initiated with any suitable priming charge.

2. A main charge consisting of 0.5 gram of a mixture of equal parts of tetranitroaniline and potassium chlorate is charged and pressed into an ordinary detonator shell. This secondary charge is then initiated with any suitable priming charge. This priming charge may be fulminate of mercury or a mixture of fulminate of mercury and a heavy metal azide or any other suitable composition.

While I have cited specific examples of nitroaromatic compounds I wish to have it

understood that in so doing the scope of my invention is not restricted to these particular explosives. The spirit of my invention includes all nitroaromatic compounds which are suitable for detonator compositions, when used in any suitable proportions mixed with oxygen carriers. It should also be understood that my invention is not limited to any particular oxygen carrying compound but includes any salt rich in oxygen which is suitable for the purpose in question.

Having described my invention, what I claim is:

1. A compound detonator consisting of a main charge and a priming charge and wherein the main charge consists of a mixture of equal parts of tetranitroaniline and potassium chlorate and wherein the priming charge consists of a mixture of fulminate of mercury and a heavy metal azide.

2. A compound detonator comprising a main charge consisting of a nitroaromatic compound and an oxygen carrier, in combination with a priming charge consisting of a mixture of a heavy metal azide and fulminate of mercury.

In testimony whereof he affixes his signature in the presence of two witnesses.

BENNETT GROTTA.

Witnesses:

RUSSELL M. COOK,  
ALLAN F. KRAFF.